

# UNITED STATES PATENT OFFICE.

GEORGE R. RICHES AND WILLIAM C. PIVER, OF HOBOKEN, NEW JERSEY.

## PROCESS OF MAKING ARSENATE OF LEAD.

1,296,557.

Specification of Letters Patent.

Patented Mar. 4, 1919.

No Drawing.

Application filed February 3, 1917. Serial No. 146,327.

To all whom it may concern:

Be it known that we, GEORGE R. RICHES, a subject of the King of Great Britain, and WILLIAM C. PIVER, a citizen of the United States, and residents of Hoboken, county of Hudson, and State of New Jersey, have invented certain new and useful Improvements in Processes of Making Arsenate of Lead, of which the following is a specification.

This invention relates to an improved method for the preparation of arsenate of lead. In carrying out our method a normal lead salt, such as lead nitrate, is caused to react in water with lead oxid and the basic lead salt thus produced is caused to react with arsenic acid.

We recognize that this type of reaction is not broadly new, but as commonly carried out it has been characterized by the disadvantages of great length of time for completion of the reaction and of coarseness of the lead arsenate upon precipitation, the lead arsenate often assuming a granular form which makes it unfit for convenient application to various uses, such as an insecticide.

The present invention comprises certain improvements, as will be hereafter set forth, in the carrying out of this type of reaction whereby the length of time necessary for the reaction of given quantities to be completed is greatly lessened and a product obtained which has a finely divided physical appearance, requiring no grinding.

In carrying out the invention we make use of straight chemical reactions (no catalyzer or material foreign to the reaction being introduced) our advantageous results being obtained generally by the temperature maintained and by the method employed in introducing the arsenic acid, certain other features also contributing to the advantageous nature of our method, as will be pointed out.

We have found that to make a batch of material the following proportions and mode of procedure are correct:

In a tank of suitable size, we add 900 gallons of lead nitrate solution of specific gravity 1.02, and to this is added 1000 lbs. of lead oxid (litharge), and the temperature of the mixture is maintained at 30 degrees to 35 degrees centigrade. To this mixture is added enough arsenic acid to convert the basic lead nitrate into arsenate of lead. The arsenic acid is of about 65 degrees

Baumé strength, and contains some nitric acid incidental to its manufacture. The arsenic acid is led into the tank through one inch pipes and mixed with the solution.

We have found that by adding the arsenic acid subsequently to the mixing of the lead nitrate and lead oxid and gradually (which is here accomplished by leading the arsenic acid into the tank through a comparatively small pipe), the time necessary for the complete reaction to take place is greatly shortened, while we also believe that the comparatively slow adding of the arsenic acid aids in the precipitation of the lead arsenate in a finely divided form.

This converts the lead compound into arsenate of lead immediately, so that when the arsenic acid has all been added, the insoluble lead arsenate is ready to be filtered off and utilized.

The reactions which take place are as follows:



The excess nitric acid forming in the final reaction, reacts upon some of the excess lead oxid to form lead nitrate:



This last reaction is made use of and calculated for the amount of lead oxid first introduced. The excess of lead oxid takes care of the nitric acid formed in the reaction of the arsenic acid with the basic lead nitrate, so that the lead arsenate just formed is not redissolved finally and the product of this reaction, lead nitrate, is used over again, after filtration of the lead arsenate, to be used in the next batch of material.

The fineness of the lead arsenate, we attribute to the temperature of the solutions while the reaction is taking place, and also the tendency of the nitric acid to dissolve the lead arsenate upon its immediate formation. We have noticed actions of this nature happening in such cases as the precipitations of arsenic, antimony and tin, as sulfids; especially the tin sulfid. If the solution of tin is on the verge of being too acid, the hydrogen sulfid will precipitate the tin sulfid, but upon the discontinuance of the stream of hydrogen sulfid, the tin sulfid particles become almost microscopic in size.

until the acid conditions of the bath adjust themselves by the decomposition of small amounts of the tin sulfids by the acid. The remaining sulfid precipitate remains suspended as minute particles.

5 The arsenate of lead exhibits the same phenomena, since when the nitric acid becomes neutralized by the lead oxid, the arsenate is left in this extremely finely divided condition.

10 What we claim is:—

1. The process of making arsenate of lead which consists in producing a solution of a basic lead salt in water and subsequently 15 adding arsenic acid thereto gradually while maintaining the mixture slightly warm.

2. The process of making arsenate of lead which consists in first mixing lead oxid and a normal salt of lead in water to produce a 20 basic lead salt and subsequently adding thereto arsenic acid gradually while maintaining the mixture slightly warm.

3. The process of making a very finely divided amorphous arsenate of lead upon 25 precipitation which consists in first heating a mixture of lead oxid and a normal lead salt in water from 30 degrees to 35 degrees centigrade until a solution of a basic lead salt is obtained and subsequently introducing arsenic acid to such mixture.

4. The process of making arsenate of lead which consists in first reacting between lead oxid and lead nitrate in water to produce basic lead nitrate, and subsequently adding 35 arsenic acid thereto, the temperature being maintained during the entire series of reactions at from 30 to 35 degrees centigrade.

5. The process of making arsenate of lead which consists in first mixing an excess of 40 lead oxid and a normal salt of lead in water at a temperature of 30 to 35 degrees centigrade to produce a basic lead salt, and subsequently adding arsenic acid thereto, the excess of lead oxid being sufficient to neu-

tralize the acid freed by the reaction of the 45 basic lead salt and arsenic acid and by its combination with said acid reproducing a desired quantity of the said normal salt of lead.

6. The process of making arsenate of lead which consists in first causing a reaction between lead oxid and a lead nitrate solution of specific gravity 1.02 in the proportions of one thousand pounds of lead oxid and nine hundred gallons of lead nitrate solution, and subsequently adding thereto sufficient arsenic acid to combine with the basic lead nitrate formed by the first reaction.

7. The process of making arsenate of lead which consists in first causing a reaction between lead oxid and a lead nitrate solution of specific gravity 1.02 at a temperature of 30 to 35 degrees centigrade, in the proportions of one thousand pounds of lead oxid and nine hundred gallons of lead nitrate 55 solution, and subsequently adding thereto sufficient arsenic acid to combine with the basic lead nitrate formed by the first reaction while maintaining the above mentioned temperature throughout the final reaction.

8. The process of making arsenate of lead, which consists in reacting upon basic lead nitrate and an excess of lead oxid with arsenic acid, introducing sufficient lead oxid in excess of the combining quantity with the 70 lead nitrate to neutralize the nitric acid produced in the reaction between the basic lead nitrate and the arsenic acid, thereby preventing the ultimate redissolving of the arsenate of lead formed, and simultaneously 75 producing nitrate of lead to be subsequently used in reacting with more oxid of lead the excess of lead oxid being sufficient in amount.

Signed at the city, county and State of 85  
New York this 31st day of January, 1917.

GEORGE R. RICHES.  
WILLIAM C. PIVER.

It is hereby certified that in Letters Patent No. 1,296,557, granted March 4, 1919, upon the application of George R. Riches and William C. Piver, of Hoboken, New Jersey, for an improvement in "Processes of Making Arsenate of Lead," errors appear in the printed specification requiring correction as follows: Page 2, line 74, claim 8, beginning with the word "introducing" strike out all to and including the word "nitrate", line 76, and insert the words *the excess of lead oxid used being sufficient in amount*; same page and claim, line 82, commencing with the word "the" strike out all to the end of the claim and insert a comma and the words *and eliminating free acid at the completion of the reaction.*; and that the said Letters Patent should be read with these corrections therein that the same may conform to the record of the case in the Patent Office.

Signed and sealed this 15th day of April, A. D., 1919.

[SEAL.]

Cl. 23—13.

F. W. H. CLAY,

*Acting Commissioner of Patents.*